

## UNITED STATES PATENT OFFICE

2,208,594

## METHOD OF DYEING HAIR

John W. Orelup, Short Hills, N. J.

No Drawing. Application March 12, 1938,  
Serial No. 195,539

8 Claims. (Cl. 167—88)

This invention relates to improvements in the dyeing of hair and more particularly to the use of non-toxic preparations for dyeing or tinting the hair.

5 At the present time there are two general methods of coloring hair. One of these is the oxidation of phénylene diamines and their derivatives, or of pyrogallol, and the other involves the use of colored sulphides and other compounds 10 of metallic salts. The methods which can be employed for application of these two classes of substances are very sharply modified by the fact that both classes are toxic. Accordingly, application 15 of these compounds by other than skilled operators is accompanied with considerable risk of injury to the person to whom the preparation is applied and even though greatest care is used in the application of these preparations to the hair, it is often impossible to avoid injurious effects.

20 It is known that application of dyes of the acidic type or direct or substantive type to the hair is unavailing to dye the hair. I have found, however, that by using fixatives which I have discovered I can cause the hair to accept such dyes with excellent results. My investigations have shown that certain condensation products of polyamines with open chain fatty acid residues are peculiarly effective to act as fixatives and to 25 cause the hair to accept ordinary textile dyes. Of the polyamines I prefer to use aliphatic amines such as the ethylene, propylene, butylene, amylene polyamines, and their alkylated derivatives, such as the dimethyl or diethyl derivatives. 30 The diamines, triamines, tetramines and pentamines of these compounds of the olefine series have been found to be useful. I particularly prefer ethylene diamine, diethylene triamine, triethylene tetramine and tetraethylene pentamine, the diethylene and triethylene compounds 35 being the ones which give optimum results.

40 For the fatty acid chain compounds which are condensed with the above mentioned polyamines I may use fatty acids or fatty acid residues which give a like product having from 6 to 20 carbon atoms in the chain, preferring the saturated acids to the unsaturated. I have found that lauric and myristic acids or cocoanut fatty acids having from 12 to 14 carbon atoms in the chain 45 give optimum results because the condensation products formed therefrom are very readily soluble.

50 While the specific action of these fixatives is not entirely understood at the present time, it is known that these condensation products are cat-

ion surface active substances. Since the affinity for hair possessed by these substances is observable, it is therefore believed that one of the effects of applying these surface active substances with long cation chains to the hair is to change the natural acidic character of the hair to basic and thus enable it to accept the acidic dye.

5 By employing any suitable non-toxic acid and direct dyes which produce desirable shades. I have been able to produce a complete range of colors which are natural in tints and which, being non-toxic, are non-injurious to the hair and scalp. Examples of dyes which give suitable shades are:

| Dye                   | Color index |
|-----------------------|-------------|
| Duro Black B          | 307         |
| Direct Fast Brown M   | 420         |
| Alizarine Brown 2R    | 167         |
| Direct Fast Orange GC | 621         |

15 I do not, however, intend to limit my invention to these examples as a great variety of other non-toxic dyes of the acid type and direct type may be employed.

20 By referring to the dyes above-mentioned and others of generally similar character as non-toxic it is to be understood that the dyes used are to be of such character that, when applied to the hair in accordance with the directions herein given, they are not injurious to the hair or scalp of the average individual. Of course, particular individuals may be allergic to one or another particular dye or class of dyes. This does not, however, make it improper to characterize such a dye as non-toxic. As compared with the highly toxic metallic salts and dyes of the phénylene diamine type which have heretofore been the only classes of dyes generally available for hair dyeing, the acid and direct dyes which I am able to use by my new process, are non-injurious and substantially non-toxic.

25 The non-toxicity of the fixatives described has been tested by feeding large amounts of the compounds such as the condensation product of C<sub>12</sub> and C<sub>14</sub> acids with triethylene tetramine to animals and it has been found that no ill effects were suffered. Likewise, skin patch tests on human beings have shown no toxicity or irritation.

30 The condensation products of these amines and the fatty acids mentioned can be prepared by known methods; for instance, by preparing the

acid chloride and condensing with the amine, or by heating the fatty acid with the amine, driving off water until the condensation is completed. The products obtained are usually of waxy consistency, disperse readily in water, and of themselves have no coloring power. They are colorless compounds having a slight, pleasant odor.

The method of procedure for dyeing the hair using these compounds is simple. A weak solution (for example 1%) of the condensation product of the fatty acid and the amine in water is prepared. This solution is applied to the hair at body temperature for a short period, such as ten minutes. The hair is then dyed by application of the dyeing solution of one of the above mentioned dyes or of any suitable non-toxic acid or direct dye, depending upon the color desired. The application of the dye should be continued for a sufficient time to secure the desired color strength, fifteen minutes being a satisfactory time in the majority of cases. The hair is then rinsed with water and the process is complete. The simplicity of the process and the fact that both the intermediate and the dye are non-toxic make it clear that no expert application is necessary.

While the above method is useful where the fixative is applied in solution, it is also within the scope of this invention that the substances could be applied in solid form, being dispensed as a cake-like mass or in semi-solid form in the nature of a paste. It is also contemplated that the fixative could be applied to the hair in conjunction with a shampoo, the shampoo, of course, being of such character as not to be inimical to the necessary properties of the fixative.

The invention, while peculiarly applicable to the dyeing of human hair on the head is not necessarily limited to that use. There is broad application for a dyeing process which is simple and entirely non-toxic in fur dyeing. A particular advantage which arises from applying this method to fur dyeing lies in the elimination of possible future complaints from the users of the fur arising from skin injuries said to result from the contact of fur with the skin of the wearer where toxic dyes have been used on the fur.

Wherever the term "hair" is employed in the claims it will be understood to mean hair on the human head or fur.

I claim:

1. The method of dyeing hair which comprises the steps of rendering the hair receptive to non-toxic organic dyes by applying thereto a cation surface active compound comprising an amide of an alkylene polyamine with a higher fatty acid component and subsequently applying a water soluble non-toxic organic dye containing negative salt forming groups.

2. The method of dyeing hair which comprises the steps of rendering the hair receptive to non-toxic organic dyes by applying thereto a cation surface active compound comprising an amide of an alkylene polyamine with a higher fatty acid component containing from six to twenty carbon atoms in the chain and subsequently applying a water soluble non-toxic organic dye containing negative salt forming groups. 5

3. The method of dyeing hair which comprises the steps of rendering the hair receptive to non-toxic organic dyes by applying thereto a cation surface active compound comprising an amide of diethylene triamine with a higher fatty acid component containing from six to twenty carbon atoms in the chain and subsequently applying a water soluble non-toxic organic dye containing negative salt forming groups. 15

4. The method of dyeing hair which comprises the steps of rendering the hair receptive to non-toxic organic dyes by applying thereto a cation surface active compound comprising an amide of triethylene tetramine with a higher fatty acid component containing from six to twenty carbon atoms in the chain and subsequently applying a water soluble non-toxic organic dye containing negative salt forming groups. 20 25

5. A composition for pretreatment in the dyeing of human hair with water soluble non-toxic organic dyes containing negative salt forming groups, said composition comprising an amide of an alkylene polyamine with a higher fatty acid component and having the property of rendering the hair receptive to said dyes. 30

6. A composition for pretreatment in the dyeing of human hair with water soluble non-toxic organic dyes containing negative salt forming groups, said composition comprising an amide of an alkylene polyamine with a higher fatty acid component containing from 6 to 20 carbon atoms 40 in the chain and having the property of rendering the hair receptive to said dyes. 35

7. A composition for pretreatment in the dyeing of human hair with water soluble non-toxic organic dyes containing negative salt forming groups, said composition comprising an amide of diethylene triamine with a higher fatty acid component containing from 6 to 20 carbon atoms 45 in the chain and having the property of rendering the hair receptive to said dyes. 50

8. A composition for pretreatment in the dyeing of human hair with water soluble non-toxic organic dyes containing negative salt forming groups, said composition comprising an amide of triethylene tetramine with a higher fatty acid component containing from 6 to 20 carbon atoms 55 in the chain and having the property of rendering the hair receptive to said dyes.

JOHN W. ORELUP.